# EUROPEAN PATENT SPECIFICATION

(11) **EP 0 051 498 B1**
(45) Date of publication and mention of the grant of the patent: **16.09.1987**
(21) Application number: 81305249.5
(22) Date of filing: 04.11.1981
(51) Int. Cl.: B28B 23/02, E04C 5/00, B32B 13/00

(54) **Process for the preparation of manufactured products based on hydraulic binders**
Verfahren zur Anfertigung von hergestellten Produkten basiert auf hydraulischer Bindemitteln
Procédé pour la préparation de produits à base de liants hydrauliques

(30) Priority: 05.11.1980 IT 2576880
(43) Date of publication of application: 12.05.1982
(73) Proprietor: Montedison S.p.A., I-20121 Milan (IT)
(72) Inventor: Grondona, Adriano, Milano (IT); Vittone, Andrea, Milano (IT)
(74) Representative: Whalley, Kevin

## Description

The present invention relates to a process for the preparation of manufactured products based on hydraulic binders, provided with a reinforcement of a fibrilled synthetic polymeric material.

It is known from Spanish patent No. 460,292 to prepare manufactured articles by superimposing a plurality of fibrilled film layers, in the form of an open net, in layers of an aqueous mixture or paste of hydraulic binder.

According to such a method there are generally used water/hydraulic binder mixtures in a weight ratio of 15:100 to 50:100, and before the drying of the manufactured product it is necessary to carry out one or more extractions under vacuum of the excess water, which extractions also contribute to the diffusion of the binder inside the net-like reinforcement layers. This method requires the use of preparation, mixing, pumping, distributing and mixture dosing equipment, and involves the difficulties connected with the hazards of clogging because of premature hardening of the hydraulic binder in suspension, and also involves drawbacks due to the need to provide ducts with a high flow rate for feeding and recovering the used water.

We are also aware of PCT Specification No. WO.80/01888 which describes a method of manufacturing construction products, and of British Specification No. GB-A-2034627 which discloses a process for producing reinforced articles made from a hydraulic material.

More particularly, PCT Specification No. WO.80/ 01888 discloses a process of manufacturing construction products comprising the steps of feeding dry constituents including a liquid-setting powder and a reinforcement thereof into a moulding zone, compacting the constituents in such zone, exposing at least one upstanding surface of the compacted constituents and applying to that surface a predetermined quantity of setting liquid, being a quantity sufficient to wet all of the compacted constituents.

British Specification No. GB-A-2034627 discloses a process for producing reinforced articles made from a hydraulic material, e.g. cement, and a fibrillated film network, e.g. polypropylene, including the steps of placing a so-called mattress formed by a multiplicity of layers of fibrillated film in a mould, applying the hydraulic material to the mattress, de-watering the hydraulic material and removing the article from the mould.

The present invention provides a process for preparing a manufactured product based on a hydraulic binder and containing a reinforcement of synthetic polymeric material, the process comprising:
mixing a hydraulic binder in the form of a dry powder with the reinforcement,
applying vibratory motion to the dry constituents, and applying water uniformly over the surface of the compacted constituents,
characterized in that hydraulic binder is distributed on at least one netlike opened film, obtained by fissuring or splitting a mono-oriented film and by stretching it crosswise, and, preferably, a plurality of such netlike opened films superimposed on each other, the quantity of water is from 12% to 30% by weight based on the weight of the binder in the dry state, and the assembly of film or films, water and binder is subjected to vibratory motion to obtain a homogeneous mixture of the water and the binder inside the net formed by the film or films and is subjected to compression.

The abovementioned drawbacks of the process according to Spanish Patent No. 460, 292 may be eliminated or at least mitigated by means of the process of the present invention, according to which there is first carried out a dry mixing between the layer or layers of fibrilled film and the hydraulic binding powder, followed by the inhibition or soaking with water of the two solid phases, in a quantity sufficient for obtaining a composite manufactured product.

The operations of (a) mixing the hydraulic binder in the form of a dry powder with the reinforcement in the form of at least one fibrilled film arranged as an open net or in the form of a plurality of such fibrilled films superimposed on each other and (b) applying vibratory motion to the dry constituents may be carried out simultaneously; the operations of (c) applying water uniformly over the surface of the compacted constituents and (d) applying vibratory motion to the assembly of film or films, water and binder may likewise be carried out simultaneously.

Before the compression operation, the assembly thus obtained by said operation (d) or by the combination of said operations (c) and (d) may be subjected to a treatment under vacuum for the removal of any excess water.

A series of said operations (a) to (d) may be repeated on the non-compressed product obtained from a preceding series of operations (a) to (d), until there is obtained a manufactured product, for example a plate, of the required thickness, the compression operation being subsequently applied to obtain the finished or end product. In such a case, the vacuum treatment may be carried out at the end of each series of operations (a) to (d), or before the final compression operation.

The fibrilled films usable in the present invention may be made of any orientable synthetic polymer, and are prepared by fissuring or splitting a mono-oriented film, for example by means of heated reliefs, points or blades, and by stretching the film thus obtained crosswise, thus conferring to it a netlike structure.

Such methods are for example described in U.S. Patent No. 3,137,746 and in British Patent Nos. 1,073,741, 1,083,847 and 1,481,520.

In order to facilitate the adhesion of the fibrilled film to the binder incorporated therein, the film may also incorporate a suitable filler, such as a zirconium compound, a diatomite, or a cement mix, as described in Italian patent application Nos. 26463/79 and 26861/79.

Convenient methods for achieving the stretching of the open-net-like fibrilled film, as well as for obtaining composite net-like structures of a plurality of super-imposed fibrilled films, usable in the present invention are described in European patent application EP-A-0 021 017.

All known hydraulic binders, such as Portland cements, aluminous cements, hydraulic limes, and chalk, may be used in the process of the present invention.

One advantage of the process according to the present invention, in comparison with the preparation from aqueous mixes of binders, is that of using only the quantity of water necessary for the development of the hydration of the binder, or a quantity only slightly greater, and consequently a considerable reduction in the installation costs and the energy consumption of the process may be achieved.

The number of superimposed fibrilled films, ' used in one distribution of the hydraulic binder according to operation (a), is preferably from 2 to 100.

The quantity by weight of fibrilled film utilized is preferably from 2% to 7.5% by weight of the weight of the hydraulic binder, considered in the dry state. The quantity of the water added in the operation (c) is from 12% to 30% by weight based on the weight of the binder in the dry state.

The invention will be further described with reference to the following illustrative Examples.

### Example 1

A mono-oriented polyprolylene film, 60 microns thick, was fibrilled by passing it over a pin-roller device of the type described in British patent No. 1,073,741, and by then opening it to form a net-like structure by a crosswise stretching equal to about 12 times the original width of the film.

Thereupon there were superimposed one over the other 15 such net-like structures, arranged with their reticular axes parallel to each other, thereby obtaining a package weighing about 96 g/ m², and sized 50 x 50 cm.

This package was then placed into a suitable mold and strewn with Portland cement powder by means of a powder-dispenser which, according to known techniques, spread uniformly over the whole 50 x 50 cm plane a quantity of 650 g of cement, while simultaneously carrying out a slight vibratory motion to promote easy penetration by the cement powder into the package.

Subsequently, the net uniformly dispersed with the cement was sprinkled uniformly by means of a set of drizzling nozzles with 130 cc of water, corresponding to a water/cement ratio of 23%.

The same operations were repeated using 4 other packages, each one consisting of 15 nets, maintaining the same cement to water ratios, and finally obtaining an assembly of 15 x 4 = ₆₀ layers of fibrilled nets mixed with 650 x 4 = 2600 g of cement and 130 x 4 = 520 cc of water.

The water was additioned with a cement super- fluidizer (Melment 10 of SKW in a 20% concentration) in a ratio of 13 g per 130 cc of water.

The assembly thus obtained was subjected to lateral vibrations by means of mechanical vibrators, andto a downward compacting action with a compacting blade connected to a vibrator, according to known techniques in the field of cement processing.

Subsequently the assembly was subjected to a vacuum of 200 mmHg for about 1 minute, thereby extracting 200 cc of water; the impregnated plate formed was thereupon removed from the mold, compressed at a pressure of 45 kg/sq.cm and finally allowed to age and harden for 28 days.

The flexural strength of the obtained hardened plate, about 6 cm thick, was then measured, according to the UNI 3948 method, thereby obtaining unitary flexural strength values equal to 348 kg/sq.cm lengthwi_{'}se (or in the direction of the fissuring of the fibrilled film), and equal to 115 kg/ cm² crosswise.

### Example 2

Into a mold, sized 50 x 50 cm, fitted with vibrators for longitudinal and transversal motion, and provided with filtering means on the underside, there was placed a package of nets obtained by opening a fibrilled polypropylene film of the same characteristics as those of the film used in the preceding example 1.

The package was formed by a total of 40 nets, arranged in groups or batches of 10 nets with their main reticular axes, derived from the fibrillation, at 90° to each other, so as to impart to the cement plate to be prepared a mechanical iso- tropy.

The package was then dispersed uniformly with 1730 g of dry Portland cement powder as in the preceding example; the mold was then subjected to a slight vibration in order to facilitate penetration of the cement into the meshes of the nets.

Thereupon the nets were sprinkled with 350 g of atomized water additioned with 35 g of Melment 10, while simultaneously maintaining the slight vibration.

The mold was then subjected to a vacuum of about 200 mmHg for about 1 minute, removing thereby about 100 cc of water and thus reducing the excess water contained in the net-cement mass to about 13% of the cement.

The plate was then compressed under a pressure of 45 kg/sq.cm and was then allowed at age and harden for 28 days. The flexural strength at break of the hardened plate, about 4 mm thick, was then measured and found to be equal to 338 kg/sq.cm in one direction and to 345 kg/sq.cm in the orthogonal direction.

## Claims

1. A process for preparing a manufactured product based on a hydraulic binder and containing a reinforcement of synthetic polymeric material, the process comprising:
mixing a hydraulic binder in the form of a dry powder with the reinforcement,
applying vibratory motion to the dry constituents, and applying water uniformly over the surface of the compacted constituents,
characterized in that hydraulic binder is distributed on at least one net-like opened film, obtained byfissuring or splitting a mono-oriented film and by stretching it crosswise, and, preferably, a plurality of such net-like opened films superimposed on each other, the quantity of water is from 12% to 30% by weight based on the weight of the binder in the dry state, and the assembly of film or films, water and binder is subjected to vibratory motion to obtain a homogeneous mixture of the water and the binder inside the net formed by the film or films and is subjected to compression.

2. A process as claimed in claim 1, characterized in that a plurality of said superimposed films comprises from 2 to 100 films.

3. A process as claimed in claim 1 or 2, characterized in that the said film or films comprise from 2% to 7.5% by weight of the weight of the hydraulic binder in the dry state.

4. A process as claimed in any of claims 1 to 3, characterized in that, at the end of the operation of subjecting the assembly of film or films, water and binder to vibratory motion, there is carried out a vacuum treatment for the removal of any excess water.

## Patentansprüche

1. Verfahren zur Herstellung eines Erzeugnisses auf Basis eines hydraulischen Bindemittels, das eine Verstärkung aus einem synthetischen polymeren Material enthält, umfassend
das Mischen eines hydraulischen Bindemittels in Form eines trockenen Pulvers mit der Verstärkung,
die Anwendung einer Vibrationsbewegung auf die trockenen Bestandteile und
das gleichmäßige Aufbringen von Wasser über die Oberfläche der verdichteten Bestandteile, dadurch gekennzeichnet, daß das hydraulische Bindemittel verteilt wird auf zumindest einen netzartig geöffneten Film, erhalten durch Spalten oder Spleißen eines monoorientierten Films und durch Strecken desselben quer bzw. kreuzweise und vorzugsweise eine Vielzahl derartiger übereinander gelagerter, netzartig geöffneter Filme, die Menge des Wassers 12 bis 30 Gew.-%, bezogen auf das Gewicht des Bindemittels in trockenem Zustand, beträgt, und die Anordnung von Film oder Filmen, Wasser und Bindemittel einer Vibrationsbewegung unterzogen wird, um eine homogene Mischung des Wassers und des Bindemittels innerhalb des durch den Film oder die Filme gebildeten Netzes zu erhalten und einer Verdichtung unterzogen wird.

2. Verfahren gemäß Anspruch 1, dadurch gekennzeichnet, daß die Vielzahl der übereinander gelagerten Filme 2 bis 100 Filme umfaßt.

3. Verfahren gemäß Anspruch 1 oder 2, dadurch gekennzeichnet, daß der Film oder die Filme 2 bis 7,5 Gew.-% des Gewichts des hydraulischen Bindemittels in trockenem Zustand umfassen.

4. Verfahren gemäß einem der Ansprüche 1 bis 3, dadurch gekennzeichnet, daß am Ende der Maßnahme, mit der die Anordnung von Film oder Filmen, Wasser und Bindemittel einer Vibrationsbewegung unterzogen wird, eine Vakuumbehandlung zur Entfernung jeglichen überschüssigen Wassers durchgeführt wird.

## Revendications

1. Un procédé de préparation d'un produit manufacturé à base de liant hydralique et contenant un renforcement en matériau polymère synthétique, ce procédé consistant en:
- le mélange d'un liant hydraulique sous la forme d'une poudre sèche avec le renforcement,
- l'application d'un mouvement vibratoire aux constituants secs, et
- l'application de l'eau uniformément à la surface des constituants compactés,

caractérisé en ce que le liant hydraulique est distribué sur au moins un film réticulé ouvert obtenu par fissuration ou fendillement d'un film mono-orienté et extension de ce film en direction transversale, et de préférence une pluralité de ces films réticulés ouverts superposés, en ce que la quantité d'eau est comprise entre 12 et 30% en poids par rapport au poids du liant à l'état sec, et en ce que l'ensemble du ou des films, de l'eau et du liant est soumis à un mouvement vibratoire pour conduire à l'obtention d'un mélange homogène de l'eau et du liant à l'intérieur du réseau formé par le ou les films, puis soumis à une compression.

2. Un procédé selon la revendication 1, caractérisé en ce que la pluralité de ces films superposés comprend de 2 à 100 films.

3. Un procédé selon la revendication 1 ou 2, caractérisé en ce que ce ou ces films comprennent de 2 à 7,5% en poids de liant hydraulique à l'état sec.

4. Un procédé selon l'une quelconque des revendications 1 à 3, caractérisé en ce qu'à la fin de l'opération de mise en vibration de l'ensemble du ou des films, de l'eau et du liant, on met en oeuvre un traitement sous vide pour l'élimination de toute eau en excès.
